

Aug. 31, 1926.

1,598,452

E. SCHURER

METHOD OF MANUFACTURING UNIFORMLY LOADED CONDUCTORS

Filed August 13, 1925



Fig. 1.



Fig. 2.

E. Schurer  
inventor

By: Marks & Clark  
Attns

## UNITED STATES PATENT OFFICE.

EUGEN SCHÜRER, OF COLOGNE-MULHEIM, GERMANY, ASSIGNOR TO FELTEN AND  
GUILLAUME CARLSWERK ACTIEN GESELLSCHAFT, OF COLOGNE-MULHEIM, GERMANY.

## METHOD OF MANUFACTURING UNIFORMLY-LOADED CONDUCTORS.

Application filed August 13, 1925, Serial No. 50,144, and in Germany September 1, 1924.

It has been found necessary when manufacturing uniformly loaded conductors used for signalling purposes, in which the loading material has to be annealed for the purpose 5 of improving its magnetic properties in the case of small magnetizing forces, to arrange that the loading strip shall not be annealed until it has been applied to the actual conductor, because otherwise the magnetic properties of the loading material would be detrimentally affected by the mechanical influences exerted when the conductor is being wound. Even when this method is adopted, special additional measures must be taken 10 in order to obtain a loading material with the best possible magnetic properties. As the heat expansion coefficient of the materials from which the loading strip is usually made is smaller than that of copper and in 15 the annealing processes hitherto adopted, the copper has been heated at the same time, the full effect of the annealing was not obtained owing to the tension caused in the loading strip as a result of the copper expanding to 20 a greater extent.

In order to obviate this drawback it has already been proposed, to interpose a thin layer of material containing carbon, such as for example paper, when winding the loading strip on to the actual conductor. By this 30 means when the conductor is annealed, the burning of the layer causes sufficient space to be left for the copper to expand, thus avoiding tension in the loading strip.

This method has the disadvantage that the magnetizable materials may absorb carbon. If this drawback is avoided by substituting a layer of inorganic substance for that containing carbon, the material forming 35 the layer combines with the copper or the magnetizable substance thus affecting the mechanical and electrical properties of the conductor.

According to the present invention a different method is adopted for obtaining the space required for the expansion of the copper, between the copper conductor and the loading strip. In this case before the loading strip is wound onto the copper line, the latter is coated with a layer of a lac which hardens uniformly, dissolves completely in certain solvents, and the thickness of which corresponds to the required space. The loading strip is then wound on over the layer

of lac, whereupon after the winding, it is 55 placed in a liquid which dissolves the lac and is then annealed in a known manner.

Figure 1 of the accompanying drawing illustrates a continuously loaded conductor according to the present invention. *a* is the 60 copper conductor, *b* the layer of lac and *c* the loading or magnetizable strip. Figure 2 illustrates the same conductor after the lac has been dissolved by the solvent.

There are a great number of lacs which 65 can be used for this purpose, for instance:

(1) Shellac-colophony lac consisting of 200 grs. shellac, 150 grs. colophony, 650 grs. spirit.

(2) Celluloid lac, consisting of (a) 200 grs. 70 acetyl cellulose, 800 grs. acetone, or (b) 100 grs. celluloid, 300 grs. amyl acetate, 300 grs. acetone, 300 grs. ether, to which 50 grs. camphor may also be added.

The lacs can be completely removed again 75 with the solvents employed, that is to say the lac referred to under (1) can be removed by means of spirit, that under (2a) by means of acetone and (2b) by a mixture consisting of equal parts of amyl acetate, acetone and 80 ether.

A further feature of the invention is the addition of small percentages of insoluble and non-inflammable constituents to the lac, these substances remaining after the treatment 85 in the solvent, between the loading strip and the copper conductor and thus forming a layer which as far as possible keeps the copper conductor in a central position inside the loading strip. These additions may for instance be fine, short asbestos fibres, mica powder and the like. 90

What I claim is:

1. A method of manufacturing uniformly loaded conductors for signalling purposes, 95 consisting in coating the conductor with a layer of lac which hardens in a uniform manner, is soluble in certain solvents and is of a suitable thickness, winding the loading strip over the conductor coated with the 100 said layer then placing the conductor in a liquid which dissolves the lac and finally annealing the conductor and loading strip.

2. A method of manufacturing uniformly loaded conductors for signalling purposes, 105 consisting in coating the conductor with a layer of lac, comprising substances which dissolve in certain solvents and small

amounts of insoluble and incombustible substances, the lac hardening in a uniform manner and being of a suitable thickness, winding the loading strip over the conductor coated with the said layer, placing the conductor in a liquid which dissolves the soluble parts of the lac, the other substances

remaining between the loading strip and the conductor and finally annealing the conductor and loading strip for the purpose set forth.

In testimony whereof I have signed my name to this specification.

EUGEN SCHÜRER.